

# UNITED STATES PATENT OFFICE.

GEORGE R. SHEVILL, OF BROOKLYN, NEW YORK; MARY E. SHEVILL EXECUTRIX OF  
SAID GEORGE R. SHEVILL, DECEASED.

## PROCESS FOR TREATING FELT CLOTH.

1,103,694.

Specification of Letters Patent.

Patented July 14, 1914.

No Drawing.

Application filed August 22, 1912. Serial No. 716,361.

To all whom it may concern:

Be it known that I, GEORGE R. SHEVILL, a citizen of the United States, residing at Brooklyn, in the county of Kings and State 5 of New York, have invented new and useful Improvements in Processes for Treating Felt Cloth, of which the following is a specification.

My invention consists of a new and improved process for preparing or sizing felt cloth or felt for hats, bonnets, slippers, hoods and other articles so that the felt when treated with my preparation will retain its shape and be firm without being made hard 10 or stiff. The felt treated with my process is particularly adaptable for making felt hats.

Felt hats have heretofore been made out of felt cloth by first sizing the cloth with either a solution of glue or shellac, or a combination 20 of both. Then when dried the felt is mulled and pressed into shape on a hot stamp die. The result of this process has been that the hat so produced is stiff and it has been impossible to make what are termed 25 soft hats in this way, because, if the solution of glue or shellac, or both, were made thin enough to leave the felt hat soft, then there would not be body or firmness enough in the hat for it to retain its shape, and felt 30 treated with glue or shellac renders the felt so hard that the felt cannot be stamped into a soft hat as can be done by my process.

Soft felt hats heretofore made have been made out of what are termed bodies, cones or 35 hoods, which are hats partially formed in the process of making the felt, or, in other words, the wool is felted into the shape of a hat or into a shape very near to a hat, so that when the cone or body or hood is given 40 a light sizing of glue or shellac, or both, the hat will hold its shape, in other words, the hats are shaped in the felting process.

By treating felt with my process it is possible to get the felt into such condition 45 that a hat may be readily stamped or blocked out from a piece of felt with the result that we have a soft felt hat made much more readily and cheaper than can be done in the way which has been heretofore practised, 50 and at the same time the hat will retain its shape in all conditions of weather and temperature.

My process consists essentially of placing about five ounces of gum tragacanth in about 55 twelve quarts of water and allowing it to

remain there until it obtains a consistency of soft soap. The felt is then immersed through this solution of gum tragacanth until the felt becomes thoroughly saturated, when it is then passed through squeeze rollers and the excess of water and gum tragacanth is eliminated by means of the squeeze rollers, or instead of passing the felt through the squeeze rollers the excess water and gum tragacanth may be thrown off by centrifugal action. 65 If it is desired to have a substance with a little more firmness than obtained by gum tragacanth a small portion of gum dammar may be added. In sizing white felt a bleach may be added if necessary, and in sizing 70 colors acids or other mordant may be added to brighten or set the color if desired or necessary.

In preparing the felt cloth for hats the sizing is made as heretofore stated by placing 75 about five ounces of gum tragacanth in about twelve quarts of water until it is of a consistency of soft soap or until it is all soft, then it is strained and put into an ordinary sizing tub and heated to any desired temperature 80 so as to permeate the cloth more completely. The felt cloth is then taken and immersed and thoroughly saturated and afterward put through the ordinary squeeze rollers attached to eliminate the excess of water 85 and then dried. When dry it is cut into the desired size and mulled, which is the term used for laying up with damp cloths; when mulled to the proper state it is then taken and pressed into the required shape in a hot 90 die in a stamp press (as is done with the old style sizing); it is then left in the die until dry. We then have a hat which instead of being hard and stiff, which is the case in all other forms of sizing, is soft and pliable, 95 and will keep its shape as well, if not better than if it had been made out of the body, hood or cone which had to be first felted or made into shape. It will be seen that by use 100 of my invention a soft hat is obtained without first making the felt into a body, hood or cone.

I do not wish to confine myself as to the time of the application of the sizing. The cloth may be treated with the sizing of gum 105 tragacanth immediately after drying and before finishing if desired, or the sizing may be put in at any stage in the process of the felting as long as care is taken not to afterward wash it out or eliminate it. When 110

so sized it will be unnecessary to size it again after the cloth is finished. The felt when treated with this process is practically impervious to water and also to heat and retains the form or shape into which it is pressed. As an example of the quantity for various weights of felt I might say that four yards of felt sixty-four inches wide and weighing about twenty-six ounces to the yard will absorb the solution of five ounces of gum tragacanth to twelve quarts of water.

I claim:—

1. The process of sizing felt cloth with gum tragacanth dissolved in water so that the gum tragacanth becomes incorporated in and a part of the felt cloth and made a part of the felt.

2. The process of sizing felt cloth with

gum tragacanth and gum dammar dissolved in water so that the gum tragacanth and gum dammar become incorporated in and form a part of the felt cloth.

3. The process of sizing felt cloth, hoods, bodies and cones with gum tragacanth and gum dammar dissolved in water so that the gum tragacanth and gum dammar become incorporated in and form part of the cloth, and adding thereto bleach for white felts and acids and mordant for colors.

In testimony whereof I have hereunto set my hand in the presence of two subscribing witnesses.

GEORGE R. SHEVILL.

Witnesses:

Wm. E. HARLAND,  
CHRIS. H. ALMSTAEDT.

---

Copies of this patent may be obtained for five cents each, by addressing the "Commissioner of Patents,  
Washington, D. C."